

# UNITED STATES PATENT OFFICE.

VALDIMAR J. MELSTED, OF WINNIPEG, MANITOBA, CANADA.

## BOILER COMPOUND.

1,210,965.

Specification of Letters Patent.

Patented Jan. 2, 1917.

No Drawing.

Application filed December 10, 1913. Serial No. 805,818.

To all whom it may concern:

Be it known that I, VALDIMAR J. MELSTED, a citizen of the United States, residing at the city of Winnipeg, in Manitoba, Canada, have invented certain new and useful Improvements in Boiler Compounds; and I do hereby declare that the following is a full, clear, and exact description of the same.

My invention relates particularly to compounds to be mixed with the water in a boiler and which cause the interior of the boiler to be coated with a substance adapted to prevent the formation of scale, and, to remove the scale in cases where it has already been formed owing to lack of a detergent.

The object of my invention is to provide a compound having metallic mercury, instead of an amalgam thereof, as its predominating element. To this end I comminute a body of mercury by agitating it with a substance adapted to subdivide it into minute globules, this comminuted mercury being used alone or mixed with suitable proportions of other well known scale detergents. The advantage of the mercury is that being in a fine state of division upon its introduction into the boiler, the finely divided particles, instead of sinking directly to the bottom and there forming a pool of mercury, adhere to the rough surface of the tubes and sheets of the boiler, gradually finding their way into cracks and crevices in the scale, and working their way to the surface of the iron. Subsequently these cracks become sealed up with fresh scale, thus preventing the access of water to the iron. A slight increase in temperature ensues, causing the mercury to expand, thus forcing off a portion of the scale. I prefer, however, to mix the comminuted mercury with other well known scale detergents such as soda carbonate, soda hydrate, tri-sodium phosphate, dextrin or tannin; and for the most economical mixture, I prefer the following proportion:—

|                        |          |
|------------------------|----------|
| Finely divided mercury | 7 parts. |
| Soda carbonate         | 30 "     |
| Sodium hydrate         | 10 "     |
| Tri-sodium phosphate   | 18 "     |
| Dextrin                | 20 "     |
| Tannin                 | 15 "     |

In the process of manufacturing the compound the mercury is first placed in a closed vessel with a liquid adapted to comminute it,

such for instance, as crude petroleum, a solution of tannic acid, or other substances which are liquid at ordinary temperatures. I will describe my invention, however, referring to petroleum: The vessel is then shaken to violently agitate the mixture and cause the mercury to be comminuted, the fine particles being individually coated and thus prevented from running together, by the tannic acid solution or crude petroleum or other substance having this function. This comminuted mercury may, as above mentioned be used alone or with other well known scale detergents. In case of the larger mixture the ingredients should be well mixed in a dry condition and then sufficient water added to form a stiff paste which may be molded into bars of convenient size which will gradually dry and harden. The molded product thus produced is placed in the water in the boiler. The compound thus produced has the advantage of removing or preventing scale and incrustation and thus also preventing loss of the heat generated and reducing to a minimum the danger of explosion.

The comminution of the mercury by means of crude petroleum or tannic acid is by far the most easy method of introducing mercury in a finely comminuted state into the compound or entering the coated particle alone into boilers.

The amount of oil or tannic acid used for breaking down the mercury does not require to be accurately proportioned, but 1 part of oil to about 20 parts of mercury, by weight, affords about the best proportion.

The comminution is accomplished by simply agitating the crude petroleum or solution of tannic acid with the mercury in a closed vessel at ordinary temperatures and at atmospheric pressure. The mercury by this method may be broken up into practically any degree of fineness; I estimate that when it is broken up to a very fine degree that the size of the individual particles of mercury do not exceed 1000 of an inch in diameter, and each individual particle is so thoroughly coated with the film of oil that it remains separate for a long period of time, such, however, is not the case when tannic acid and mercury is used as the particles join each other and assume their original state when not agitated.

When the mercury is comminuted with crude petroleum it can be introduced into

a boiler to permit them to adhere to the scaly surfaces and on account of the extreme fineness of the particles they will adhere to the rough surfaces of the tubes and boiler  
5 and remain in suspension long enough without being compounded with other ingredients and enter cracks in the scale, gradually working their way toward the iron; while a very small proportion will find its way to  
10 the bottom of the boiler.

What I claim is as follows:—

1. A boiler compound comprising a comminuted mixture of mercury in its metal-

lic state and a separating substance in a liquid state at ordinary atmospheric temperature.

2. A boiler compound consisting of a mixture of comminuted metallic mercury and petroleum.

In testimony whereof I have signed my name to this specification in the presence of two witnesses.

VALDIMAR J. MELSTED.

Witnesses:

JOSEPH YATES,  
HENRY A. V. GREEN.